# EUROPEAN PATENT SPECIFICATION

(11) **EP 3 216 888 B1**
(45) Date of publication and mention of the grant of the patent: **02.06.2021**
(21) Application number: 15857850.0
(22) Date of filing: 16.10.2015
(51) Int. Cl.: C22C 38/00, C22C 38/58, C22C 38/02, C22C 38/06, C22C 38/50

(54) **USE OF A DUAL-PHASE STAINLESS STEEL MATERIAL FOR DIFFUSION BONDING**
VERWENDUNG EINES ZWEIPHASIGEN EDELSTAHLMATERIALS ZUM DIFFUSIONSSCHWEISSEN
UTILISATION D'UN ACIER INOXYDABLE À DEUX PHASES POUR UN PROCESSUS DE SOUDAGE PAR DIFFUSION

(30) Priority: 05.11.2014 JP 2014225576
(43) Date of publication of application: 13.09.2017
(73) Proprietor: Nisshin Steel Co., Ltd., Chiyoda-ku Tokyo 100-8366 (JP)
(72) Inventor: SUGAMA, Atsushi, Sakai-shi Osaka 592-8332 (JP); KAGEOKA, Kazuyuki, Shunan-shi Yamaguchi 746-8666 (JP); HORI, Yoshiaki, Shunan-shi Yamaguchi 746-8666 (JP); IMAKAWA, Kazunari, Shunan-shi Yamaguchi 746-8666 (JP); OKU, Manabu, Sakai-shi Osaka 592-8332 (JP)
(74) Representative: Papula Oy
(86) International application number: PCT/JP2015/079342
(87) International publication number: WO 2016/072244

(56) References cited:
- EP-A1- 1 396 552
- JP-A- H07 256 468
- JP-A- 2003 089 851
- JP-A- 2004 131 743
- JP-A- 2010 090 456
- JP-A- 2013 011 437
- JP-A- 2013 103 271
- JP-A- 2013 173 181
- JP-A- 2014 185 369
- JP-A- 2014 190 664
- US-A1- 2009 072 009

## Description

### TECHNICAL FIELD

The present invention relates to the use of a dual-phase stainless steel material for diffusion bonding, and to a method for producing a diffusion bonded product by performing diffusion bonding using a dual-phase stainless steel material for diffusion bonding.

### BACKGROUND ART

One method of bonding stainless steel materials to each other includes a diffusion bonding method. A stainless steel diffusion bonded product assembled by diffusion bonding has been applied in various applications such as heat exchangers, machine components, fuel cell components, home appliance components, plant components, ornament constituent members, and building materials. The diffusion bonding method includes an "insert material inserting method" of inserting an insert material into a bonding interface, and performing bonding by solid phase diffusion or liquid phase diffusion; and a "direct method" of directly bringing surfaces of both stainless steel materials into contact with each other, and performing diffusion bonding.

The insert material inserting method is advantageous in that it is capable of realizing certain diffusion bonding in a relatively simple manner. However, this method becomes disadvantageous as compared with a direct method for the following reasons. That is, an insert material is used, thus leading to an increase in costs, and also a bonding portion is formed of metal which is different from that forms a base material, thus leading to deterioration of corrosion resistance. On the other hand, it is commonly said to be difficult for the direct method to obtain sufficient bonding strength as compared with the insert material inserting method. However, this direct method includes the possibility to become advantageous in that it can reduce production costs, so that various methods have been studied. For example, Patent Document 1 discloses technology in which the amount of S in a stainless steel is set at 0.01% by weight or less and also diffusion bonding is performed in a non-oxidizing atmosphere at a predetermined temperature, thereby avoiding deformation of the material, thus leading to an improvement in diffusion bondability of a stainless steel material. Patent Document 2 discloses a method using a stainless steel foil material whose surface is imparted with unevenness by a pickling treatment. Patent Document 3 discloses a method using, as a material to be bonded, a stainless steel whose Al content is suppressed so that an alumina film, which causes inhibition of diffusion bonding, is less easily to be formed during diffusion bonding. Patent Document 4 discloses a method in which diffusion is promoted using a stainless steel foil imparted with deformation by cold working. Patent Documents 5 and 6 describe a ferritic stainless steel for direct diffusion bonding, the component composition of which is optimized.

Patent Document 1: Japanese Unexamined Patent Application, Publication No. S62-199277
Patent Document 2: Japanese Unexamined Patent Application, Publication No. H02-261548
Patent Document 3: Japanese Unexamined Patent Application, Publication No. H07-213918
Patent Document 4: Japanese Unexamined Patent Application, Publication No. H09-279310
Patent Document 5: Japanese Unexamined Patent Application, Publication No. H09-99218
Patent Document 6: Japanese Unexamined Patent Application, Publication No. 2000-303150
Patent Document 7: Japanese Unexamined Patent Application, Publication No. 2013-103271
Patent Document 8: Japanese Unexamined Patent Application, Publication No. 2013-173181
Patent Document 9: Japanese Unexamined Patent Application, Publication No. 2013-204149
Patent Document 10: Japanese Unexamined Patent Application, Publication No. 2013-204150

EP 1396552 describes a martensite/ferrite dual-phase stainless steel strip useful as steel belts.

### DISCLOSURE OF THE INVENTION

### Problems to be Solved by the Invention

The above-mentioned bonding technology enabled implementation of diffusion bonding of a stainless steel material even when using a direct method. However, from the industrial point of view, the direct method is yet to be taken root as the mainstream of a diffusion bonding method of the stainless steel material. The main reason is the fact that it is difficult to achieve both two issues, for example, security of reliability in the bonding portion, such as bonding strength or adhesiveness, and suppression of a load in the production, such as bonding device or bonding time. According to conventional technical knowledge, in order that the bonding portion to be produced by the direct method, there is a need to employ a step requiring a large production load, such as a step in which a bonding temperature is set at high temperature of higher than 1,100°C, or a step in which high surface pressure is imparted by hot press, HIP, or the like, so that it was impossible to avoid an increase in costs due to the step. When an attempt is made to carry out diffusion bonding of a stainless steel material by the direct method under the same workload as in a conventional insert material inserting method, it is difficult to sufficiently secure reliability of the bonding portion in the current situation.

Thus, there has been proposed a method for producing a diffusion bonded product by a direct method, which can be carried out under the same workload as in a conventional insert material inserting method without applying special high-temperature heating or high surface pressure by making use of a driving force when a ferrite phase is transformed into an austenite phase during diffusion bonding (Patent Document 7) or a driving force of crystal grain growth (Patent Document 8). There has also been proposed a method in which an amount of a surface oxide of a stainless steel material to be allowed to undergo diffusion bonding is reduced as much as possible, thereby enhancing diffusion bondability (Patent Documents 9 and 10). To secure good bondability, there is a need for these methods to regulate surface roughness before bonding of a stainless steel material to be used. Therefore, there is a need to further improve bondability in a stainless steel material to be used in a diffusion bonded product.

An object of the present invention is to provide a stainless steel material suitable for diffusion bonded molding, diffusion bondability of which is further improved without being influenced by the extent of surface roughness.

### Means for Solving the Problems

The present inventors have found that, by controlling an average crystal grain size before diffusion bonding, an amount of γmax, and creep elongation of a dual-phase stainless steel material having a dual-phase structure composed of at least two phases of a ferrite phase, a martensite phase, and an austenite phase, good diffusion bondability can be obtained without being influenced by surface roughness of the steel material. Specifically, the present invention is defined by the independent claims. Embodiments are described in dependent claims.

### Effects of the Invention

According to the present invention, a dual-phase stainless steel having a dual-phase structure composed of at least two phases of a ferrite phase, a martensite phase, and an austenite phase is provided with an average crystal grain size and γmax before diffusion bonding, and creep elongation at a bonding temperature in an optimum range, whereby, a stainless steel material having excellent diffusion bondability is used for diffusion bonding, thus providing a diffusion bonded molding which exhibits a good bonding interface. The total content of Ti and Al is suppressed, thereby obtaining a diffusion bonded molding having improved diffusion bondability.

### BRIEF DESCRIPTION OF THE DRAWINGS

Fig. 1 is a drawing showing a measurement test piece used in a bondability test.

### PREFERRED MODE FOR CARRYING OUT THE INVENTION

Embodiments of the present invention will be described below. The present invention is not limited to the description thereof.

It is considered that diffusion bonding by a direct method of a stainless steel material is completed by simultaneous proceeding of three types of processes, for example, a process (i) in which unevenness of a bonding surface undergoes deformation leading to adhesion, thus increasing a bonding area of the bonded position, a process (ii) in which a surface oxide film of the steel material before bonding disappears at the adhered position, and a process (iii) in which a residual gas in voids as the unbonded portion reacts with a base material, according to a conventional technique.

Heretofore, the present inventors have studied so as to avoid deterioration of productivity, which creates an industrial obstacle, by regulating a base material component, components included in a passive film, and surface roughness of a bonding surface, focusing attention on the process (ii) mentioned above. However, it is sometimes difficult to secure industrially stable bondability even when the step (ii) mentioned above is controlled. Therefore, numerous studies have been performed on a steel material for obtaining stable bondability considering the step (i) mentioned above. As a result, it has been found that, when a stainless steel to be allowed to undergo diffusion bonding is a dual-phase stainless steel having a dual-phase structure, it is extremely effective to reduce a crystal grain size before diffusion bonding.

### [Dual-Phase Structure]

Stainless steels are commonly classified into an austenitic stainless steel, a ferritic stainless steel, a martensitic stainless steel, and the like based on a metal structure at normal temperature. A "dual-phase structure" of the present invention has a metal structure composed of at least two phases of a ferrite phase, a martensite phase, and an austenite phase. The "dual-phase stainless steel material" of the present invention means a steel which has such a dual-phase structure, and exhibits an austenitic-ferritic two-phase structure within a bonding temperature range. Stainless steels classified into a ferritic stainless steel and a martensitic stainless steel are sometimes included in such a two-phase stainless steel.

In the present invention, in order to realize diffusion bonding by a direct method at low temperature under low surface pressure, a dual-phase stainless steel having a dual-phase structure composed of at least two phases of a ferrite phase, a martensite phase, and an austenite phase is used as a stainless steel material to be allowed to undergo diffusion bonding. Regarding this stainless steel, within a temperature range where diffusion bonding proceeds, a ferrite phase and a martensite phase are partially transformed into an austenite phase to form a two-phase structure composed of an austenite phase and a ferrite phase. There will easily take place creep deformation which is considered to cause grain boundary sliding as a result of maintenance of a fine structure due to suppression of crystal grain growth of each phase in the two-phase structure at high temperature. As a result, easy deformation is promoted at the unevenness portion of a bonding surface, leading to an increase in a bonding area of the bonded portion, thus enabling diffusion bonding by a direct method at low temperature under low surface pressure.

The dual-phase stainless steel material used according to the present invention can be used as both or one of stainless steel materials which are directly brought into contact with each other and integrated by diffusion bonding. It is possible to apply, as a mating material to be integrated, in addition to the stainless steel material of the present invention, other types of two-phase steels, types of austenitic steels in which an austenite single-phase is formed within a heating range of diffusion bonding, types of ferritic steels in which a ferrite single-phase is formed within the heating range, and the like.

### [Component Composition]

In the dual-phase stainless steel which is used according to the present invention, there is no need to be particular about component elements other than Ti and Al from the viewpoint of diffusion bondability, and it is possible to employ various component compositions according to the uses. The present invention is directed to an austenitic-ferritic two-phase structure within a temperature range where diffusion bonding proceeds, so that there is a need to employ a steel having a component composition in which ymax represented by the formula (a) mentioned below satisfies a range of 10 to 90. It is possible to exemplify, as a specific component composition range, the followings.

Component composition including, in % by mass: C: 0.2% or less, Si: 1.0% or less, Mn: 3.0% or less, P: 0.05% or less, S: 0.03% or less, Ni: 10.0% or less, Cr: 10.0 to 30.0%, N: 0.3% or less, Ti: 0.15% or less, and Al: 0.15% or less, with the remainder being Fe and inevitable impurities, wherein the total amount of Ti and Al is 0.15% or less.

Component composition further comprising, in % by mass: one or two or more elements of Nb: 4.0% or less, Mo: 0.01 to 4.0%, Cu: 0.01 to 3.0%, and V: 0.03 to 0.15%. Component composition further including, in % by mass: B: 0.0003 to 0.01%.

Components included in the stainless steel material will be described below.

C improves strength and hardness of a steel by solid solution strengthening. Meanwhile, an increase in C content causes deterioration of workability and toughness of the steel, so that the C content is 0.2% by mass or less, and preferably 0.08% by mass or less.

Si is an element used for deoxidation of the steel. Meanwhile, excessive Si content causes deterioration of toughness and workability of the steel. Thus, a firm surface oxide film is formed to inhibit diffusion bondability. Therefore, the Si content is 1.0% by mass or less, and preferably 0.6% by mass or less.

Mn is an element which improves high-temperature oxidation properties. Meanwhile, excessive Mn content allows the steel to undergo work hardening, leading to deterioration of cold workability of the steel. Therefore, the Mn content is 3.0% by mass or less.

P is an inevitable impurity element and enhances intergranular corrosion properties and also causes deterioration of toughness of the steel. Therefore, the P content is 0.05% by mass or less, and preferably 0.03% by mass or less.

S is an inevitable impurity element and causes deterioration of hot workability of the steel. Therefore, the S content is 0.03% by mass or less.

Ni is an austenite formation element and has a function of improving corrosion resistance of the steel in a reducing acid environment. Meanwhile, excessive Ni content makes an austenite phase stable, thus failing to suppress the growth of a ferrite crystal, so that a stable austenite single-phase is formed to suppress the growth of the ferrite crystal. Therefore, the Ni content is 10.0% or less.

Cr is an element which forms a passive film to impart corrosion resistance. Therefore, the Cr content is 10.0 to 30.0% by mass.

N is an inevitable impurity element and causes deterioration of cold workability, so that the content thereof is 0.3% by mass or less.

Ti has a function of fixing C and N and is therefore an element effective in improving corrosion resistance and workability. Al is often added as a deoxidizing agent. Meanwhile, Ti and Al are easily oxidizable elements, so that Ti oxide and Al oxide included in an oxide film on a surface of the steel material are less likely to be reduced in a heat treatment of vacuum diffusion bonding. Therefore, numerous Ti oxide or Al oxide may cause prevention of proceeding of the process (ii) mentioned above during diffusion bonding, so that the Ti content is 0.15% by mass or less, while the Al content is 0.15% by mass or less, and preferably 0.05% by mass. The total content of Ti and Al is set at 0.15% by mass or less, and preferably 0.05% by mass or less.

Nb is an element which forms carbide or carbonitride to refine crystal grains of the steel, thus exerting the effect of enhancing the toughness. Meanwhile, excessive Nb content causes deterioration of workability of the steel, so that the Nb content is 4.0% by mass or less.

Mo is an element which has a function of improving corrosion resistance without reducing the strength. Excessive Mo content causes deterioration of workability of the steel, so that the Mo content is 0.01 to 4.0% by mass.

Cu is an element which is effective in improving corrosion resistance, and also has a function of forming a ferrite phase. Meanwhile, excessive Cu content causes deterioration of workability of the steel, so that the Cu content is 0.01 to 3.0% by mass.

V is an element which contributes to an improvement in workability and toughness of the steel by fixing solid-soluted C as carbide. Meanwhile, excessive content of a V element causes deterioration of productivity, so that the V content is 0.03 to 0.15%.

B is an element which contributes to an improvement in corrosion resistance and workability by fixing N. Meanwhile, excessive content of a B element causes deterioration of hot workability of the steel, so that the B content is 0.0003 to 0.01%.

It is possible to apply, as a dual-phase stainless steel having the chemical composition mentioned above, a steel in which γmax represented by the formula (a) mentioned below is 10 to 90: $γ max = 420 C - 11.5 Si + 7 Mn + 23 Ni - 11.5 Cr - 12 Mo + 9 Cu - 49 Ti - 47 Nb - 52 Al + 470 N + 189$ where an element symbol of C, Si, and the like in the above formula (a) means the content (% by mass) of each element.

ymax is an indicator which represents an amount (% by volume) of an austenite phase formed when heated and retained at about 1,100°C. When γmax is 100 or more, it is possible to regard as types of austenitic steels in which an austenite single-phase is formed. When ymax is 0 or less, it is possible to regard as types of ferrite steels in which a ferrite single-phase is formed. Regarding the dual-phase stainless steel of the present invention, when γmax is 10 to 90, an austenitic-ferritic two-phase is formed within a temperature range where diffusion bonding proceeds, and two phases mutually suppress crystal grain growth at high temperature, so that it is effective for obtaining a fine crystal structure. ymax is more preferably 50 to 80.

### [Average Crystal Grain Size before Bonding]

The more the grain structure of the dual-phase stainless steel of the present invention becomes fine, more quickly the process (i) mentioned above can be allowed to proceed. Therefore, the average crystal grain size before bonding is 20 µm or less, and more preferably 10 µm or less.

### [Surface Roughness]

Regarding the dual-phase stainless steel including fine crystal grains of the present invention, the process (i) mentioned above quickly proceeds, so that the process (ii) mentioned above exerts a small influence and there is low possibility that bondability is restricted by the extent of surface roughness Ra. If surface roughness of the stainless steel material to be allowed to undergo diffusion bonding increases, disappearance of an oxide film in the process (ii) mentioned above tends to become late. Therefore, a surface of the stainless steel material is preferably smooth, and surface roughness Ra is preferably 0.3 µm or less.

### [Method for Producing Diffusion bonded product]

Regarding the stainless steel material of the present invention, a diffusion bonded product having good bondability is obtained by performing vacuum diffusion bonding using a direct method. Specific diffusion bonding treatment is as follows, for example, diffusion bonding can be allowed to proceed by heating and retaining in a furnace under the conditions of a pressure of 1.0 × 10⁻² Pa or less (preferably 1.0 × 10⁻³ Pa or less) and a dew point of -40°C or lower at 900 to 1,100°C in a state of being directly contacted under a contact surface pressure of 0.1 to 1.0 MPa. The retention time can be adjusted within a range of 0.5 to 3 hours.

### EXAMPLES

Examples of the present invention will be described below. The present invention is not limited to the following Examples, and can be carried out within the scope of the present claims by making appropriate modifications.

A stainless steel with the chemical composition shown in Table 1 was melted by vacuum melting (30 kg). The steel ingot thus obtained was forged into a 30 mm thick plate and then hot-rolled at 1,230°C for 2 hours to obtain a 3.0 mm thick hot rolled sheet. Then, annealing, pickling, and cold rolling was performed to obtain a 1.0 mm thick cold rolled sheet. Thereafter, the cold rolled sheet was subjected to an annealing treatment mentioned below to produce a cold rolled annealed sheet, which was used as a test material.

**[Table 1]**

| Phase | Steel material | C | Si | Mn | P | S | Ni | Cr | Cu | Mo | Al | Ti | Nb | V | B | N |
|---|---|---|---|---|---|---|---|---|---|---|---|---|---|---|---|---|
| *α* + M | FM-1 | 0.064 | 0.54 | 0.31 | 0.01 | 0.002 | 1.90 | 16.37 | 0.04 | 0.04 | 0.004 | 0.004 | - | - | - | 0.011 |
| | FM-2 | 0.095 | 0.16 | 0.50 | 0.02 | 0.003 | 0. 10 | 16.28 | - | - | 0.007 | - | - | - | - | 0.010 |
| | FM-3 | 0.080 | 0.20 | 0.44 | 0.03 | 0.005 | 0.11 | 17.02 | 0.02 | 0.01 | 0.090 | 0.033 | - | - | 0.0015 | 0.015 |
| | FM-4 | 0.018 | 0.38 | 0.49 | 0.02 | 0.004 | 0.09 | 16.82 | 0.01 | 0.01 | 0.002 | 0.001 | - | - | - | 0.009 |
| *α* + *γ* | FA-1 | 0.010 | 0.44 | 0.57 | 0.02 | 0.004 | 6.55 | 23.55 | 0.46 | 3.21 | 0.055 | - | 0.18 | 0.08 | - | 0.109 |
| | FA-2 | 0.013 | 0.48 | 0.62 | 0.01 | 0.009 | 6.44 | 24.54 | 0.46 | 2.88 | 0.080 | - | - | 0.06 | 0.0020 | 0.150 |
| *α* | F-1 | 0.009 | 0.33 | 0.99 | 0.02 | 0.010 | 0.13 | 18.32 | 0.17 | 2.00 | 0.017 | 0.010 | 0.61 | 0.05 | - | 0.009 |
| *γ* | A-1 | 0.060 | 0.44 | 1.04 | 0.02 | 0.003 | 8.06 | 18.05 | - | 0.11 | - | 0.010 | - | - | - | 0.015 |
| M | M-1 | 0.133 | 0.45 | 0.60 | 0.03 | 0.011 | 0.09 | 12.34 | 0.06 | 0.02 | 0.001 | - | - | - | 0.0009 | 0.014 |

| | | | | | | | | | | | | | | | | |
|---|---|---|---|---|---|---|---|---|---|---|---|---|---|---|---|---|
| (*α* : Ferrite phase M: Martensite phase *γ*: Austenite phase) | | | | | | | | | | | | | | | | |

Plural steel materials are shown in Table 1. The metal structure before diffusion bonding of each of FM-1 steel to FM-4 steel is composed of a ferritic-martensitic two-phase (α + M phase). The metal structure before diffusion bonding of each of FA-1 steel and FA-2 steel is composed of a ferritic-austenitic two-phase (α + γ phase). The metal structure before diffusion bonding of F-1 steel is composed of a ferrite single-phase (α phase). The metal structure before diffusion bonding of A-1 steel is composed of an austenite single-phase (γ phase). The metal structure before diffusion bonding of M-1 steel is composed of a martensite single-phase (M phase). By changing an annealing temperature of each steel sheet after cold rolling within a range of 900°C to 1,200°C, test materials each having a different average crystal grain size were obtained. To examine an influence of surface roughness, test materials each having different surface roughness Ra were obtained by changing a finishing treatment of a cold rolled annealed sheet using a part of a steel sheet.

### (Average Crystal Grain Size)

An average crystal grain size before diffusion bonding (µm) of a steel sheet was measured by a quadrature procedure as mentioned below. A metal structure of a sheet thickness cross-section parallel to a cold rolling direction was observed with respect to a continuous area of 1 mm² or more, and then the number of crystal grains included in a unit area was calculated using a quadrature procedure. Thereafter, an average area per one crystal grain was determined and a value obtained by raising variable the average area to the power of 1/2 was used as an average crystal grain size.

### (Surface Roughness)

Regarding surface roughness Ra (µm), surface roughness Ra in a direction perpendicular to a rolling direction was measured using a surface roughness measuring instrument (SURFCOM2900DX; manufactured by TOKYO SEIMITSU CO., LTD.).

### (Creep Elongation)

Creep elongation was measured by the method mentioned below. A JIS13B test piece was cut out from each steel sheet and a ϕ5 mm hole was made at the center of one grip. A making-off line (50 mm in length, between gauge marks) was formed on the test piece, and then the test piece was attached to a high temperature tensile testing machine so that the grip with a hole faces downward. After temperature rise until the temperature between the gauge marks becomes 1,000°C and soaking at the same temperature for 15 minutes, a wire made of SUS310S provided with a weight calculated so as to apply stress of 1.0 MPa was attached to the hole of the grip, followed by retaining for 0.5 hour. The wire made of SUS310S was removed from the test piece and cooled to normal temperature by air cooling. Then, the length L between gauge marks was measured and (L-50)/50 × 100 was calculated as creep elongation (%).

### (Bondability Test)

Plane test pieces measuring 20 mm × 20 mm were cut out from each steel sheet and diffusion bonding was performed by the following method. Two test pieces made of the same steel material were laminated in a state where surfaces of the test pieces come into contact with each other. Using a jig with a weight, surface pressure to be applied to a contact surface of these two test pieces was adjusted to 0.1 MPa. Hereinafter, the plane test piece thus laminated is referred to as a "steel material". Those in which the steel materials are laminated are referred to as a "laminate". Then, the jig and the laminate were placed in a vacuum furnace. Vacuuming was performed until the pressure reaches initial vacuum degree of 1.0 × 10⁻³ to 1.0 × 10⁻⁴ Pa and the temperature was raised to 1,000°C over about 1 hour, followed by retaining at the same temperature for 2 hours. After transferring to a cooling chamber, cooling was performed. During cooling, the vacuum degree was maintained up to 900°C and then an Ar gas was introduced, followed by cooling to about 100°C or lower in an Ar gas atmosphere under 90 kPa. Regarding the laminate after completion of the heat treatment, using a ultrasonic thickness gage (manufactured by OLYMPUS CORPORATION; Model 35DL), the thickness was measured at 49 measurement points formed at 3 mm pitch on a laminate surface measuring 20 mm × 20 mm as shown in Fig. 1. A probe diameter was set at 1.5 mm. When a measured value of the sheet thickness at certain measurement point exhibits the total sheet thickness of two steel materials, it is possible to consider that both steel materials are integrated with each other by diffusion of atoms at the position of an interface between both steel materials corresponding to the measurement point. Meanwhile, when a measured value of the sheet thickness is different from the total sheet thickness of two steel materials, it is possible to consider that the unbonded portion (defect) exists at the position of an interface between both steel materials corresponding to the measurement point. A correspondence relation between a cross-sectional structure of the laminate after a heating treatment and the measurement results obtained by this measurement technique was examined. As a result, it has been confirmed that it is possible to accurately evaluate an area ratio of the bonded portion in a contact area by the value obtained by dividing the number of measurement points where the measurement results exhibited the total sheet thickness of both steel materials by the total number of measurement 49 (hereinafter this is referred to as a "bonding ratio"). Diffusion bondability was evaluated by the following evaluation criteria.
A: Bonding ratio of 100% (excellent)
B: Bonding ratio of 90 to 99% (good)
C: Bonding ratio of 60 to 89% (fairly good)
D: Bonding ratio of 0 to 59% (bad)

As a result of various studies, sufficient strength of the diffusion bonded portion was secured and also sealability (property not causing leakage of a gas through communicating defects) between both members is good in ratings A and B, so that ratings A and B were considered as passing.

An average crystal grain size and ymax after cold rolling annealing of each steel, surface roughness, creep elongation, and bondability are shown in Table 2.

**[Table 2]**

| Category | Steel material | *γ* max | Average crystal grain size (*µ* m) | Creep elongation (%) | Surface roughness R a (*µ*m) | Bondability | Remarks (phase) |
|---|---|---|---|---|---|---|---|
| Inventive Example 1 | FM-1 | 71.9 | 9 | 1.42 | 0.40 | A | *α* + M |
| Inventive Example 2 | FM-1 | 71.9 | 15 | 0.80 | 0.56 | B | |
| Inventive Example 3 | FM-2 | 50.0 | 18 | 0.42 | 0.22 | B | |
| Inventive Example 4 | FM-3 | 31.0 | 11 | 0.95 | 0.12 | B | |
| Inventive Example 5 | FA-1 | 77.5 | 12 | 1.11 | 0.33 | A | *α* + *γ* |
| Inventive Example 6 | FA-1 | 77.5 | 16 | 0.65 | 0.49 | B | |
| Comparative Example 1 | FM-1 | 71.9 | 35 | 0.11 | 0.28 | C | *α* + M |
| Comparative Example 2 | FM-4 | 8.3 | 16 | 0.12 | 0.43 | C | |
| Comparative Example 3 | FA-1 | 77.5 | 26 | 0.14 | 0.27 | C | *α* + *γ* |
| Comparative Example 4 | FA-2 | 95.1 | 18 | 0.09 | 0.15 | C | |
| Comparative Example 5 | F-1 | -60.0 | 15 | 0.08 | 0.41 | D | *α* |
| Comparative Example 6 | F-1 | -60.0 | 41 | 0.05 | 0.32 | D | |
| Comparative Example 7 | F-1 | -60.0 | 41 | 0.05 | 0.05 | B | |
| Comparative Example 8 | A-1 | 199.5 | 12 | 0.17 | 0.31 | D | *γ* |
| Comparative Example 9 | A-1 | 199.5 | 25 | 0.13 | 0.04 | B | |
| Comparative Example 1 0 | M-1 | 110.9 | 35 | 0.12 | 0.54 | D | M |

| | | | | | | | |
|---|---|---|---|---|---|---|---|
| (Underlined numerical value shows a value deviating from the scope of the present invention.) | | | | | | | |

As shown in Table 2, in Inventive Examples 1 to 6, a bonding ratio was 90% or more and good diffusion bondability was exhibited even at comparatively low temperature, for example, 1,000°C under low surface pressure, for example, 0.1 MPa. In Inventive Examples 1 to 6, good diffusion bondability was exhibited regardless of the extent of surface roughness Ra, and there was no influence of surface roughness. Since dual-phase stainless steel material having a structure of the present invention does not cause deterioration of diffusion bondability even when surface roughness increases, it is apparent that diffusion bondability thereof is not restricted to surface property of the steel material.

To the contrary, in Comparative Examples 1 to 10, an average crystal grain size, γmax, and creep elongation deviated from the scope of the present invention, leading to small deformation of the unevenness portion of the bonding surface within a two-phase high temperature range, thus failing to increase the bonding area at the bonded position. Therefore, numerous bonding ratios are less than 80% and rated fairly bad or bad. Regarding ferrite single-phase steels of Comparative Examples 5 to 7 and austenite single-phase steels of Comparative Examples 8 to 9, according to a change in bonding ratio depending on the surface roughness Ra, Comparative Example 7 and Comparative Example 9 with very small surface roughness exhibited a bonding ratio of 90% or more. Meanwhile, other Comparative Examples exhibited large surface roughness, and a bonding ratio decreased. As is apparent from the above results, in a single-phase steel, large surface roughness leads to bad bonding ratio, so that diffusion bondability is restricted by surface roughness.

## Claims

1. Use of a dual-phase stainless steel material for diffusion bonding, a metal structure before diffusion bonding having a dual-phase structure composed of at least two phases of a ferrite phase, a martensite phase, or an austenite phase, wherein
the dual-phase structure has an average crystal grain size of 20 µm or less,
ymax represented by the formula (a) mentioned below is 10 to 90, and
creep elongation is 0.2% or more when a load of 1.0 MPa is applied at 1,000°C for 0.5 hour,
the stainless steel material comprises, in % by mass: C: 0.2% or less, Si: 1.0% or less, Mn: 3.0% or less, P: 0.05% or less, S: 0.03% or less, Ni: 10.0% or less, Cr: 10.0 to 30.0%, N: 0.3% or less, Ti: 0.15% or less, and Al: 0.15% or less;
optionally comprises, in % by mass: one or two or more elements of Nb: 4.0% or less, Mo: 0.01 to 4.0%, Cu: 0.01 to 3.0%, and V: 0.03 to 0.15%,
optionally comprises, in % by mass: B: 0.0003 to 0.01%; wherein the remainder is Fe and inevitable impurities, wherein the total amount of Ti and Al is 0.15% or less: $γ max = 420 C - 11.5 Si + 7 Mn + 23 Ni - 11.5 Cr - 12 Mo + 9 Cu - 49 Ti - 47 Nb - 52 Al + 470 N + 189$ where an element symbol in the formula (a) mentioned above denotes the content (% by mass) of each element, and wherein an average crystal grain size is measured according to the method as specified in the description.

2. The use according to claim 1, wherein the stainless steel is used for direct diffusion bonding.

3. The use according to claim 1 or 2, wherein the stainless steel is used for vacuum diffusion bonding using a direct method.

4. A method for producing a diffusion bonded product by performing diffusion bonding using a dual-phase stainless steel material for diffusion bonding, a metal structure before diffusion bonding having a dual-phase structure composed of at least two phases of a ferrite phase, a martensite phase, or an austenite phase, wherein
the dual-phase structure has an average crystal grain size of 20 µm or less,
ymax represented by the formula (a) mentioned below is 10 to 90, and
creep elongation is 0.2% or more when a load of 1.0 MPa is applied at 1,000°C for 0.5 hour,
the stainless steel material comprises, in % by mass: C: 0.2% or less, Si: 1.0% or less, Mn: 3.0% or less, P: 0.05% or less, S: 0.03% or less, Ni: 10.0% or less, Cr: 10.0 to 30.0%, N: 0.3% or less, Ti: 0.15% or less, and Al: 0.15% or less;
optionally comprises, in % by mass: one or two or more elements of Nb: 4.0% or less, Mo: 0.01 to 4.0%, Cu: 0.01 to 3.0%, and V: 0.03 to 0.15%,
optionally comprises, in % by mass: B: 0.0003 to 0.01%; wherein the remainder is Fe and inevitable impurities, wherein the total amount of Ti and Al is 0.15% or less: $γ max = 420 C - 11.5 Si + 7 Mn + 23 Ni - 11.5 Cr - 12 Mo + 9 Cu - 49 Ti - 47 Nb - 52 Al + 470 N + 189$ where an element symbol in the formula (a) mentioned above denotes the content (% by mass) of each element, and wherein an average crystal grain size is measured according to the method as specified in the description.

5. The method according to claim 4, wherein performing direct diffusion bonding using the stainless steel material.

6. The method according to claim 4 or 5, wherein performing vacuum diffusion bonding using a direct method using the stainless steel material.

## Patentansprüche

1. Verwendung eines zweiphasigen rostfreien Stahlmaterials zum Diffusionsschweißen, wobei eine Metallstruktur vor dem Diffusionsschweißen eine zweiphasige Struktur aufweist, die aus mindestens zwei Phasen einer Ferritphase, einer Martensitphase oder einer Austenitphase zusammengesetzt ist, wobei
die zweiphasige Struktur eine durchschnittliche Kristallkorngröße von 20 µm oder weniger aufweist,
ymax, dargestellt durch die unten erwähnte Formel (a), 10 bis 90 beträgt, und
die Kriechdehnung 0,2% oder mehr beträgt, wenn eine Belastung von 1,0 MPa bei 1.000°C für 0,5 Stunden aufgebracht wird,
wobei das rostfreie Stahlmaterial in Masse-% umfasst: C: 0,2% oder weniger, Si: 1,0% oder weniger, Mn: 3,0% oder weniger, P: 0,05% oder weniger, S: 0,03% oder weniger, Ni: 10,0% oder weniger, Cr: 10,0 bis 30,0%, N: 0,3% oder weniger, Ti: 0,15% oder weniger, und Al: 0,15% oder weniger; optional umfasst, in Masse-%: ein oder zwei oder mehr Elemente von Nb: 4,0% oder weniger, Mo: 0,01 bis 4,0%, Cu: 0,01 bis 3,0%, und V: 0,03 bis 0,15%,
optional umfasst, in Masse-%: B: 0,0003 bis 0,01%;
wobei der Rest aus Fe und unvermeidbaren Verunreinigungen besteht,
wobei die Gesamtmenge von Ti und Al 0,15% oder weniger ist: $γ max = 420 C - 11,5 Si + 7 Mn + 23 Ni - 11,5 Cr - 12 Mo + 9 Cu - 49 Ti - 47 Nb - 52 Al + 470 N + 189$ wobei ein Elementsymbol in der oben erwähnten Formel (a) den Gehalt (Masse-%) jedes Elements angibt, und wobei eine durchschnittliche Kristallkorngröße nach dem in der Beschreibung spezifizierten Verfahren gemessen wird.

2. Die Verwendung nach Anspruch 1, wobei der rostfreie Stahl für direktes Diffusionsschweißen verwendet wird.

3. Die Verwendung nach Anspruch 1 oder 2, wobei der rostfreie Stahl für Vakuum-Diffusionsschweißen nach einem direkten Verfahren verwendet wird.

4. Ein Verfahren zur Herstellung eines diffusionsgeschweißten Produktes durch Diffusionsschweißen unter Verwendung eines zweiphasigen rostfreien Stahlmaterials zum Diffusionsschweißen, wobei eine Metallstruktur vor dem Diffusionsschweißen eine zweiphasige Struktur aufweist, die aus mindestens zwei Phasen einer Ferritphase, einer Martensitphase oder einer Austenitphase zusammengesetzt ist, wobei
die zweiphasige Struktur eine durchschnittliche Kristallkorngröße von 20 µm oder weniger aufweist,
ymax, dargestellt durch die unten erwähnte Formel (a), 10 bis 90 beträgt, und
die Kriechdehnung 0,2% oder mehr beträgt, wenn eine Belastung von 1,0 MPa bei 1.000°C für 0,5 Stunden aufgebracht wird,
wobei das rostfreie Stahlmaterial in Masse-% umfasst: C: 0,2% oder weniger, Si: 1,0% oder weniger, Mn: 3,0% oder weniger, P: 0,05% oder weniger, S: 0,03% oder weniger, Ni: 10,0% oder weniger, Cr: 10,0 bis 30,0%, N: 0,3% oder weniger, Ti: 0,15% oder weniger, und Al: 0,15% oder weniger; optional umfasst, in Masse-%: ein oder zwei oder mehr Elemente von Nb: 4,0% oder weniger, Mo: 0,01 bis 4,0%, Cu: 0,01 bis 3,0%, und V: 0,03 bis 0,15%,
optional umfasst, in Masse-%: B: 0,0003 bis 0,01%;
wobei der Rest aus Fe und unvermeidbaren Verunreinigungen besteht,
wobei die Gesamtmenge von Ti und Al 0,15% oder weniger ist: $γ max = 420 C - 11,5 Si + 7 Mn + 23 Ni - 11,5 Cr - 12 Mo + 9 Cu - 49 Ti - 47 Nb - 52 Al + 470 N + 189$ wobei ein Elementsymbol in der oben erwähnten Formel (a) den Gehalt (Masse-%) jedes Elements angibt, und wobei eine durchschnittliche Kristallkorngröße nach dem in der Beschreibung spezifizierten Verfahren gemessen wird.

5. Das Verfahren nach Anspruch 4, wobei direktes Diffusionsschweißen unter Verwendung des rostfreien Stahlmaterials durchgeführt wird.

6. Das Verfahren nach Anspruch 4 oder 5, wobei Vakuum-Diffusionsschweißen nach einem direkten Verfahren unter Verwendung des rostfreien Stahlmaterials durchgeführt wird.

## Revendications

1. Utilisation d'un matériau en acier inoxydable biphasé pour le soudage par diffusion, une structure métallique avant le soudage par diffusion ayant une structure biphasée composée d'au moins deux phases parmi une phase de ferrite, une phase de martensite ou une phase d'austénite, où
la structure biphasée a une taille moyenne des grains cristallins inférieure ou égale à 20 µm,
ymax représenté par la formule (a) mentionnée ci-dessous est compris entre 10 et 90, et
l'allongement par fluage est supérieur ou égal à 0,2% lorsqu'une charge de 1,0 MPa est appliquée à 1000°C pendant 0,5 heure,
le matériau en acier inoxydable comprend, en % en masse : C : 0,2% ou moins, Si : 1,0% ou moins, Mn : 3,0% ou moins, P : 0,05% ou moins, S : 0,03% ou moins, Ni : 10,0% ou moins, Cr : 10,0 à 30,0%, N : 0,3% ou moins, Ti : 0,15% ou moins, et Al : 0,15% ou moins ;
comprend éventuellement, en % en masse : un ou deux élément(s) ou plus parmi Nb : 4,0% ou moins, Mo : 0,01 à 4,0%, Cu : 0,01 à 3,0%, et V : 0,03 à 0,15%,
comprend éventuellement, en % en masse : B : 0,0003 à 0,01% ;
où le reste est Fe et des impuretés inévitables, où la quantité totale de Ti et d'Al est inférieure ou égale à 0,15% : $γ max = 420 C - 11,5 Si + 7 Mn + 23 Ni - 11,5 Cr - 12 Mo + 9 Cu - 49 Ti - 47 Nb - 52 Al + 470 N + 189$ où un symbole d'élément dans la formule (a) mentionnée ci-dessus indique la teneur (% en masse) de chaque élément, et
où une taille moyenne des grains cristallins est mesurée selon le procédé tel que spécifié dans la description.

2. Utilisation selon la revendication 1, dans laquelle l'acier inoxydable est utilisé pour le soudage par diffusion directe.

3. Utilisation selon la revendication 1 ou 2, dans laquelle l'acier inoxydable est utilisé pour le soudage par diffusion sous vide en utilisant un procédé direct.

4. Procédé de production d'un produit soudé par diffusion en réalisant un soudage par diffusion en utilisant un matériau en acier inoxydable biphasé pour le soudage par diffusion, une structure métallique avant le soudage par diffusion ayant une structure biphasée composée d'au moins deux phases parmi une phase de ferrite, une phase de martensite ou une phase d'austénite, où
la structure biphasée a une taille moyenne des grains cristallins inférieure ou égale à 20 µm,
ymax représenté par la formule (a) mentionnée ci-dessous est compris entre 10 et 90, et
l'allongement par fluage est supérieur ou égal à 0,2% lorsqu'une charge de 1,0 MPa est appliquée à 1000°C pendant 0,5 heure,
le matériau en acier inoxydable comprend, en % en masse : C : 0,2% ou moins, Si : 1,0% ou moins, Mn : 3,0% ou moins, P : 0,05% ou moins, S : 0,03% ou moins, Ni : 10,0% ou moins, Cr : 10,0 à 30,0%, N : 0,3% ou moins, Ti : 0,15% ou moins, et Al : 0,15% ou moins ;
comprend éventuellement, en % en masse : un ou deux élément(s) ou plus parmi Nb : 4,0% ou moins, Mo : 0,01 à 4,0%, Cu : 0,01 à 3,0%, et V : 0,03 à 0,15%,
comprend éventuellement, en % en masse : B : 0,0003 à 0,01% ;
où le reste est Fe et des impuretés inévitables, où la quantité totale de Ti et d'Al est inférieure ou égale à 0,15% : $γ max = 420 C - 11,5 Si + 7 Mn + 23 Ni - 11,5 Cr - 12 Mo + 9 Cu - 49 Ti - 47 Nb - 52 Al + 470 N + 189$ où un symbole d'élément dans la formule (a) mentionnée ci-dessus indique la teneur (% en masse) de chaque élément, et
où une taille moyenne des grains cristallins est mesurée selon le procédé tel que spécifié dans la description.

5. Procédé selon la revendication 4, comprenant la réalisation d'un soudage par diffusion directe en utilisant le matériau en acier inoxydable.

6. Procédé selon la revendication 4 ou 5, comprenant la réalisation d'un soudage par diffusion sous vide en utilisant un procédé direct utilisant le matériau en acier inoxydable.
